

# UNITED STATES PATENT OFFICE.

CHARLES BAECHLER, OF LOMPOC, CALIFORNIA.

## PROCESS FOR MAKING PHOTOSTEREOTYPES FOR TYPOGRAPHIC PRINTING-PRESSES.

1,088,512.

Specification of Letters Patent.

Patented Feb. 24, 1914.

No Drawing.

Application filed March 28, 1913. Serial No. 757,367.

*To all whom it may concern:*

Be it known that I, CHARLES BAECHLER, a citizen of the United States, and a resident of Lompoc, in the county of Santa Barbara 5 and State of California, have invented a new and Improved Process for Making Photostereotypes for Typographic Printing-Presses, of which the following is a full, clear, and exact description.

10 The invention relates to the process of making printing blocks directly from any negative or film, by employing bichromated gelatin or glue and a screen or chemical grain to form the printing block.

15 In the collotype or artotype process, the printing is done from a gelatin plate and must be printed on specially constructed presses, similar to a lithograph. These processes, however, do not involve the process 20 of constructing a typographic printing block. My process differs from the above, in that I cast my printing blocks directly from the glue or gelatin plate, and do not use the gelatin or glue for printing.

25 In order to construct the printing block or casting, a mold is required, and this mold is made from bichromated gelatin and a chemical grain or screen. The ordinary gelatin plate now generally used can also be 30 employed to constitute the mold. The chlorid and bromid of silver contained in these plates combined with bichromatic salts previously impregnated in the plates constitute the mold to make the casting and 35 mit the casting of a typographic printing block, from which numberless printed impressions can be easily obtained.

40 In order to cast directly upon the bichromated gelatin or glue plates described, after they have been properly exposed to daylight or artificial light under any common photographic negative and screen and then swelled up by the use of water to the desired relief, I employ a composition of sulfur and black 45 lead in various proportions and melted together by the minimum degree of heat required to melt sulfur. This composition or mixture is then cast directly upon the relief of the mentioned glue mold or plate, and a 50 suitable backing is also disposed thereon, thus constituting the desired block for typographic printing. The backing mentioned is preferably formed of several layers of wire or iron nails and wire netting of about 55  $\frac{1}{4}$ -inch,  $\frac{1}{2}$ -inch, or  $\frac{3}{4}$ -inch mesh, and the said backing reinforces the black lead and sulfur

block and prevents the same from cracking or breaking. The relative proportions of sulfur and black lead constituting the composition consist of approximately four parts 60 of sulfur to one part of black lead. With this proportion a coarse surface is obtained, desirable for ordinary newspaper printing and the like. Where a highly polished surface is desired the proportionate amounts of 65 sulfur and black lead are slightly varied. The mentioned composition of sulfur and black lead can be employed also as a base for electro or stereotype plates or any other forms or kinds of plates used in photo- 70 engraving, such as copper or zinc plates.

A chemical grain for photo-mechanical printing blocks can be produced in several ways, one of which I will describe herewith.

After the bichromated gelatin mold has 75 been properly exposed under a negative and developed so that it is prepared to be cast upon with molten sulfur and black lead, I sprinkle a quantity of dry, finely powdered chlorid of sodium on the said gelatin mold. 80 After the resulting block or cut is separated from the mentioned mold, the fine particles of sodium are found to be embedded in the surface of the printing block and these particles are dissolved by the action of water, 85 thus leaving minute depressions in the surface of the cut or printing block and the said depressions constitute a chemical grain.

By means of the process described, it is 90 easily possible to produce a printing block in less than an hour, without the use of any special machinery, and it will be understood that the scope of my invention is substantially defined in the appended claims.

Having thus described my invention, I 95 claim as new and desire to secure by Letters Patent:

1. The herein described process for producing printing blocks, consisting in forming a mold composed of bichromated gelatin having a chemical grain or screen, and coating the face of the mold with a compound of sulfur and black lead to derive a casting, the said casting being adapted to constitute a surface for the said printing 100 block.

2. The herein described process for producing printing blocks, consisting in forming a mold composed of glue having a chemical grain or screen, and coating the face of 110 the mold with a composition of sulfur and black lead, to derive a casting, the said cast-

ing being adapted to constitute a surface for the said printing block.

3. The herein described process for producing printing blocks, consisting in impregnating the face of a gelatin or glue plate with bichromated salts, forming a mold from said bichromated gelatin or glue plate having a chemical grain or screen, and coating the face of the mold with a mixture of melted sulfur and black lead to form a casting, the said casting being adapted to constitute a surface for the said printing block.

4. The herein described process for producing printing blocks, consisting in impregnating the face of a gelatin or glue plate with a mixture of chlorid of silver, bromid of silver and bichromate salts, forming a mold from said bichromated gelatin or glue plate having a chemical grain or screen, and coating the face of said mold with a composition of sulfur and black lead to form a casting.

5. The herein described process for producing printing blocks, consisting in forming a mold composed of bichromated gelatin or glue having a chemical grain or

screen, and coating the face of the mold with a compound of sulfur and black lead reinforced by a backing to derive a casting, the said casting being adapted to constitute a surface for the said printing block.

6. The herein described process for producing printing blocks, consisting in impregnating gelatin or glue with bichromated salts, forming a mold from said bichromated gelatin or glue, applying a soluble salt in fine powder to the surface of the mold to produce a chemical grain, coating the face of the mold with a mixture of melted sulfur and black lead to form a casting having the soluble particles embedded in the surface thereof, and then dissolving the soluble particles, the said casting being adapted to constitute a surface for the said printing block.

In testimony whereof I have signed my name to this specification in the presence of two subscribing witnesses.

CHARLES BAECHLER.

Witnesses:

T. A. HOFFMAN,  
W. B. HOFFMAN.